

## UNITED STATES PATENT OFFICE

2,613,194

## FIBER FORMING SOLUTIONS

Alfred B. Craig, Dayton, Ohio, assignor, by mesne assignments, to The Chemstrand Corporation, a corporation of Delaware

No Drawing. Application September 26, 1950,  
Serial No. 186,909

14 Claims. (Cl. 260—308)

1

This invention relates to new and valuable fiber spinning solutions. More specifically the invention relates to dispersions of solvents and blended mixtures of acrylonitrile polymers and vinylpyridine polymers which have improved low viscosities and high solid content.

It is well-known that polyacrylonitrile and copolymers of acrylonitrile and other polymerizable mono-olefinic monomers are excellent fiber forming compositions. The polymers of 80 per cent or more acrylonitrile and up to 20 per cent of other monomers, such as vinyl acetate, methyl methacrylate, methyl acrylate, styrene, vinylidene chloride, and methacrylonitrile are capable of production into fibers with superior physical properties. Although fibers so prepared have superior tensile properties, desirable elongation, and excellent stability over a wide range of physical and chemical conditions, they are subject to certain inherent disabilities which greatly restrict their utility as general purpose fibers. For example, these compositions and the fibers prepared therefrom do not have sufficient dye affinity to enable the development of satisfactory colored fibers. Furthermore, many of the compositions are difficult to prepare in suitable solutions, due to viscosity increases, gellation and the development of cloudy solutions when conventional fiber spinning procedures are practiced.

In copending application, Serial No. 158,332, filed April 26, 1950, by David W. Chaney and Howard M. Hoxie, there are described and claimed new fiber spinning compositions, which have the desirable fiber properties of the prior art acrylonitrile polymers, but which have unusual receptivity for dyestuffs. In accordance with this procedure the undyeable acrylonitrile polymers are blended with polymers which are inherently better dye acceptors. The blended polymer not only acquires satisfactory dye receptivity but is also found to have an unusually superior thermostability. In the spinning of the blended polymers it has been found that heterogeneous cloudy solutions, partial gellation, increases in viscosity and other irregularities are frequently encountered.

The fundamental purpose of this invention is to provide means of the improved spinning of the blended polymers. A further purpose of the invention is to provide a means of reducing the viscosity and increasing the spinnability of the solution without lowering the solid content, and conversely, increasing the solid content of a spinning solution without increasing the viscosity. A still further purpose is to eliminate the cloudi-

2

ness and other heterogeneous irregularities in spinning solutions.

It has been found that blended polymers of substantial proportions of the non-dyeable acrylonitrile polymers and minor proportions of a vinylpyridine or alkyl substituted vinylpyridine polymer may be dissolved in conventional solvents for fiber forming acrylonitrile polymers to produce solutions of unusual quality with respect to homogeneity and spinnability if the solutions are made in the presence of a minor proportion of sulfuric acid, for example from 0.01 to 3.00 weight per cent based on the solution. Preferred practice utilizes from 0.05 to 1.00 per cent. Such mixtures have been found to have lower viscosities and complete freedom from turbidity as compared to the same solutions not containing the sulfuric acid. Although the invention is particularly applicable to blended vinylpyridine polymers, where heterogeneous properties are frequent and the minimization thereof a common problem, the invention is also useful with respect to copolymers of acrylonitrile and vinylpyridine, particularly the copolymers of 90 to 98 per cent acrylonitrile and from two to ten per cent of a vinylpyridine or an alkyl substituted vinylpyridine.

The invention is applicable to both blends and copolymers which are comprised of from two to ten per cent of a vinylpyridine or an alkyl substituted vinylpyridine, said percentage being based on the total monomers of which the copolymer or blend of copolymers are comprised. The blends may have as the principal polymer from 50 to 98 per cent of a copolymer of 90 or more per cent acrylonitrile and minor proportions of monomers copolymerizable therewith. The other blend constituent is a polyvinylpyridine or a copolymer of 30 or more per cent of a vinylpyridine or alkyl substituted vinylpyridine and up to 70 per cent of another copolymerizable monomer. The two components of the blended copolymers are proportioned such as to provide the required quantity of acrylonitrile and reactive vinylpyridine.

The vinylpyridine in both the copolymers and blend copolymers may be any vinylpyridine or alkyl substituted vinylpyridine, for example 2-vinylpyridine, 3-vinylpyridine, 4-vinylpyridine, 2-vinyl-4-ethylpyridine, 2-vinyl-3-methylpyridine, 5-vinyl-2-methylpyridine, 2-vinyl-5-ethylpyridine, 2-vinyl-4-methylpyridine, 3-vinyl-5-ethylpyridine and any other vinylpyridine containing alkyl substituents wherein the alkyl radical has up to four carbon atoms.

The dyeable copolymers, or dyeable blended copolymers, may have in addition to the functional components, acrylonitrile and a vinylpyridine, one or more other components derived from monomers such as vinyl acetate, and other vinyl esters of carboxylic acids having up to four carbon atoms, vinyl chloroacetate, methyl methacrylate, methyl acrylate and other alkyl acrylates and alkyl methacrylates wherein the alkyl radical has up to four carbon atoms, diethyl maleate, diethyl fumarate and other alkyl maleates and fumarates wherein the alkyl radical has up to four carbon atoms, styrene and other vinyl substituted aromatic hydrocarbons, vinylidene chloride and methacrylonitrile. These non-functional monomers may be present as a third monomer with acrylonitrile and a vinylpyridine in a terpolymeric system, or they may be used in the blended composition either as a comonomer with acrylonitrile in the principal polymer or as a comonomer with a vinylpyridine in the blending polymer.

The principal acrylonitrile polymers and copolymers thereof may be prepared in any of the manners well-known to the art. Of particular utility are the emulsion or dispersion polymerizations which take place in an aqueous medium in the presence of water-soluble peroxy compounds or other free radical type of catalysts and with a suitable dispersing agent. Such polymerizations may take place at elevated temperatures utilizing reflux conditions to eliminate the heat of polymerization or the reaction may be conducted by the "Redox" methods in lower temperatures. It is also conventional to use regulators, for example the various mercaptans, such as tert.-dodecyl mercaptan, mercapto acetic acid, and the esters of mercapto acetic acid. The separation of the acrylonitrile polymers from the aqueous medium may be accomplished by filtration or decantation followed by drying in the manner well-known to the art.

The vinylpyridine polymers may be by mass polymerization methods, solution polymerization methods, or aqueous emulsion procedures, the latter being the preferred manner of preparation. The preferred procedure involves the use of efficient emulsion stabilizing agents for the purpose of preventing agglomeration with the polymer particles. The details of polymerization procedure and separation of the polymer from the reaction medium may be practiced by any of the numerous methods known to the art.

The fiber forming acrylonitrile polymer and vinylpyridine polymers are physically blended by a wide variety of procedures. If desired the emulsions or dispersions of polymers in aqueous media, just as received from the polymerization reactors may be blended. Physical mixtures of the separated solid polymers may also be utilized. A preferred manner of preparing the mixtures involves the dispersion of the polymers, or the emulsions thereof, in a solvent, with the distillation or evaporation of the water, if present in proportions large enough to interfere with the complete dissolution of the solid polymers. In the preparation of the blends in the presence of a conventional solvent, or preferably N,N-dimethylacetamide, from which the fiber spinning will ultimately take place, frequently non-homogeneous, cloudy dispersions are obtained. Other solvents which may be used in the practice of this invention are butyrolactone, N,N-dimethylformamide, ethylene carbonate, maleic anhydride, N,N-dimethylmethoxyacetamide, succinic anhydride, and  $\alpha$ -cyanoacetamide.

In accordance with the practice of this invention minor proportions of sulfuric acid are added. It has been found that the addition of 0.01 per cent to five per cent by weight (based on the solvent) of sulfuric acid will eliminate the turbidity and produce clear, transparent, light-colored polymer solutions. The treatment has also been found to cause a marked reduction in the viscosity, thereby enabling the spinning with higher solid content in the spinning solutions or spinning at low temperatures. Improvements in dye receptivity and dye fastness were noted. Further details of the invention are set forth with respect to the following specific examples:

15

*Example 1*

A series of fiber spinning solutions were prepared by blending 84 per cent by weight of a copolymer of 97 per cent acrylonitrile and three per cent vinyl acetate with 16 per cent of a copolymer of 50 per cent vinyl pyridine and 50 per cent acrylonitrile in sufficient N,N-dimethylacetamide to yield an 18 per cent solids solution. The resulting solutions were found to be turbid and to have a viscosity of 117 poises at 50° C. Several samples of this spinning solution were treated with varying proportions of sulfuric acid. The following table demonstrates that improvements in viscosity and clarity of the solution are obtained by the addition of sulfuric acid to the spinning solution.

| Wt. Percent H <sub>2</sub> SO <sub>4</sub> in Solution | Clarity of Solution   | Viscosity Poises 50° C. |
|--------------------------------------------------------|-----------------------|-------------------------|
| 35 .00                                                 | Turbid                | 117                     |
| .031                                                   | Cloudy                | 99                      |
| .062                                                   | Clear, light in color | 92                      |
| .125                                                   | do                    | 95                      |
| 1.50                                                   | Cloudy                | 90                      |

40

*Example 2*

The effect of sulfuric acid on spinning solutions of higher solids content was demonstrated by preparing a 24.5 per cent solids content spinning solution of the copolymer blend described in the preceding example. The untreated solution was found to be cloudy and to have a viscosity of 371 poises at 50° C. The addition of 0.2 cc. of sulfuric acid per 300 grams of solution clarified the solution entirely and reduced the viscosity to 324 poises at 50° C.

50

*Example 3*

A mixture of 622.5 parts by weight of N,N-dimethylacetamide, 112.2 parts of a copolymer of 97 per cent of acrylonitrile and three per cent vinyl acetate and 15.3 parts of a copolymer of 50 per cent of pyridine and 50 per cent acrylonitrile was prepared by stirring the mixture at 80° C. for one hour. Sulfuric acid in the amount of 0.38 part by weight was added thereto, thereby forming a clear and homogeneous spinning solution. The solution was spun through a spinneret having 30 apertures each 0.005 inch in diameter into a mixture of 60 per cent N,N-dimethylacetamide and 40 per cent water. The fiber so produced was then washed with water, stretched 150 per cent while wet and then 422 per cent in a steam atmosphere. The fiber so prepared had a tenacity of 3.2 g./d., seven per cent elongation and was found to have an excellent acceptance to Wool Fast Scarlet Dye.

60

65

*Example 4*

Using the procedure described in Example 1, a copolymer of 97 percent acrylonitrile and three

70

75

percent vinyl acetate was prepared. Two samples were dissolved in N,N-dimethylacetamide to form 20.8 percent solids solutions. One of the sample solutions was treated with 0.125 percent H<sub>2</sub>SO<sub>4</sub>, and then mixed mixed thoroughly. The viscosities of both treated and untreated solutions were determined at 50° C. The untreated solution had a viscosity of 353 poises, whereas the acid treated solution had a viscosity of 253 poises.

*Example 5*

A copolymer of 92 percent by weight of acrylonitrile and eight percent of vinylpyridine was dissolved to the extent of 18 percent by weight in N,N-dimethylacetamide. The solution was found to have a viscosity of 235 poises at 50° C. By adding 0.19 percent of sulfuric acid, the viscosity was found to be reduced to 180 poises.

*Example 6*

A series of blends of various proportions of a copolymer of 97 percent acrylonitrile and three percent vinyl acetate, and a copolymer of 50 percent vinylpyridine and 50 percent acrylonitrile were prepared, dissolved in N,N-dimethylacetamide and treated with sulfuric acid in different proportions. The solutions so obtained were all spun into fibers which had excellent dye acceptance. The following table shows the variation in proportions used and the nature of the spinning solution:

| Wt. Percent Vinylpyridine | Wt. Percent Sulfuric Acid |                        |
|---------------------------|---------------------------|------------------------|
| 6                         | 0.05                      | Clear and homogeneous. |
| 6                         | 0.30                      | Do.                    |
| 8                         | 0.06                      | Do.                    |
| 8                         | 1.25                      | Cloudy.                |
| 4                         | 0.20                      | Clear and homogeneous. |

These experiments demonstrate that when more than one percent of sulfuric acid is used, cloudy solutions may be formed. This lack of clarity does not affect the spinnability of the solution. Improvements in lowered viscosity are found at all concentrations.

The invention is defined by the following claims.

What I claim is:

1. A fiber spinning solution comprising a solvent for fiber-forming acrylonitrile polymers, polymer of monomeric substances of which from two to ten percent of the total monomer is a vinylpyridine and at least 80 percent is acrylonitrile, and from 0.01 to 3.0 percent by weight (based on the solution) of sulfuric acid.

2. A fiber spinning solution comprising a solvent for fiber-forming acrylonitrile polymers, polymer of monomeric substances of which from two to ten percent of the total monomer is a vinylpyridine and at least 80 percent is acrylonitrile, in polymeric form, and from 0.05 to 1.0 percent by weight (based on the solution) of sulfuric acid.

3. A fiber spinning solution comprising a solvent for fiber-forming acrylonitrile polymers, a copolymer of 90 to 98 percent acrylonitrile and from two to ten percent vinylpyridine, and from 0.01 to 3.0 percent by weight (based on the solution) of sulfuric acid.

4. A fiber spinning solution comprising a solvent for fiber-forming acrylonitrile polymers, a blend of a polymer of at least 90 percent acrylonitrile and a polymer of at least 30 percent of vinylpyridine, said polymers being so propor-

tioned as to provide from two to ten percent of vinylpyridine in polymeric form in the blended polymer, and from 0.01 to 3.0 percent by weight (based on the solution) of sulfuric acid.

5. A fiber spinning composition comprising a N,N-dimethylacetamide solution of polymer of monomeric substances of which from two to ten percent of the total monomer is a vinylpyridine and at least 80 percent is acrylonitrile, and from 0.01 to 3.0 percent by weight (based on the solution) of sulfuric acid.

6. A fiber spinning composition comprising a N,N-dimethylacetamide solution of polymer of monomeric substances of which from two to ten percent of the total monomer is a vinylpyridine and at least 80 percent is acrylonitrile in polymeric form, and from 0.05 to 1.0 percent by weight (based on the solution) of sulfuric acid.

7. A fiber spinning composition comprising a N,N-dimethylacetamide solution of a copolymer of 90 to 98 percent acrylonitrile and from two to ten percent of vinylpyridine and from 0.01 to 3.0 percent by weight (based on the solution) of sulfuric acid.

8. A fiber spinning composition comprising a N,N-dimethylacetamide solution of a copolymer of 90 to 98 percent acrylonitrile and from two to ten percent of vinylpyridine, and from 0.05 to 1.0 percent by weight (based on the solution) of sulfuric acid.

9. A fiber spinning composition comprising a N,N-dimethylacetamide solution of a blend of a polymer of at least 90 percent acrylonitrile and a polymer of at least 30 percent vinylpyridine, said polymers being blended in such proportions so as to produce polymer having from two to ten percent of vinylpyridine in polymeric form, and from 0.01 to 3.0 percent by weight (based on the solution) of sulfuric acid.

10. A fiber spinning composition comprising a N,N-dimethylacetamide solution of a blend of polymer of at least 90 percent acrylonitrile and a polymer of at least 30 percent vinylpyridine, said polymers being blended in such proportions so as to produce polymer having from two to ten percent vinylpyridine in polymeric form, and from 0.05 to 1.0 percent by weight (based on the solution) of sulfuric acid.

11. A fiber spinning solution comprising a solvent for fiber-forming acrylonitrile polymers, a blend of a polymer of at least 90 percent acrylonitrile and up to ten percent of a monomer of the group consisting of vinyl acetate and other vinyl esters of carboxylic acids having up to four carbon atoms, vinylchloroacetate, methyl methacrylate, methyl acrylate, other alkyl acrylates and methacrylates wherein the alkyl radical has up to four carbon atoms, styrene, other vinyl substituted aromatic hydrocarbons, vinylidene chloride, diethyl fumarate, diethyl maleate, other alkyl fumarates and alkyl maleates wherein the alkyl radical has up to four carbon atoms and methacrylonitrile; and a polymer of at least 30 percent of vinylpyridine and up to 70 percent of acrylonitrile; and from 0.01 to 3.0 percent by weight (based on the solution) of sulfuric acid said blend of polymers being so proportioned so as to provide vinylpyridine to the extent of from two to ten percent of the total polymerized monomer.

12. A fiber spinning solution comprising a solvent for fiber-forming acrylonitrile polymers, a blend of a polymer of at least 90 percent acrylonitrile and up to ten percent of a monomer of the group consisting of vinyl acetate and other vinyl esters of carboxylic acids having up to four car-

bon atoms, vinylchloroacetate, methyl methacrylate, methyl acrylate, other alkyl acrylates and methacrylates wherein the alkyl radical has up to four carbon atoms, styrene, other vinyl substituted aromatic hydrocarbons, vinylidene chloride, diethyl fumarate, diethyl maleate, other alkyl fumarates and alkyl maleates wherein the alkyl radical has up to four carbon atoms and methacrylonitrile; and a polymer of at least 30 percent of vinylpyridine and up to 70 percent of acrylonitrile; and from 0.05 to 1.0 percent by weight (based on the solution) of sulfuric acid said blend of polymers being so proportioned so as to provide vinylpyridine to the extent of from two to ten percent of the total polymerized monomer.

13. A fiber spinning composition comprising a N,N-dimethylacetamide solution of a blend of a polymer of at least 90 percent acrylonitrile and up to ten percent of a monomer of the group consisting of vinyl acetate and other vinyl esters of carboxylic acids having up to four carbon atoms, vinylchloroacetate, methyl methacrylate, methyl acrylate, other alkyl acrylates and methacrylates wherein the alkyl radical has up to four carbon atoms, styrene, other vinyl substituted aromatic hydrocarbons, vinylidene chloride, diethyl fumarate, diethyl maleate, other alkyl fumarates and alkyl maleates wherein the alkyl radical has up to four carbon atoms and methacrylonitrile; and a polymer of at least 30 per cent of vinylpyridine and up to 70 percent of acrylonitrile; and from 0.01 to 3.0 percent by weight (based on the solution) of sulfuric acid said blend of polymers be-

ing so proportioned so as to provide vinylpyridine to the extent of from two to ten percent of the total polymerized monomer.

14. A fiber spinning composition comprising a N,N-dimethylacetamide solution of a blend of a polymer of at least 90 percent acrylonitrile and up to ten percent of a monomer of the group consisting of vinyl acetate and other vinyl esters of carboxylic acids having up to four carbon atoms, vinylchloroacetate, methyl methacrylate, methyl acrylate, other alkyl acrylates and methacrylates wherein the alkyl radical has up to four carbon atoms, styrene, other vinyl substituted aromatic hydrocarbons, vinylidene chloride, diethyl fumarate, diethyl maleate, other alkyl fumarates and alkyl maleates wherein the alkyl radical has up to four carbon atoms and methacrylonitrile; and a polymer of at least 30 percent of vinylpyridine and up to 70 percent of acrylonitrile; and from 0.05 to 1.0 percent by weight (based on the solution) of sulfuric acid said blend of polymers being so proportioned so as to provide vinylpyridine to the extent of from two to ten percent of the total polymerized monomer.

ALFRED B. CRAIG.

#### REFERENCES CITED

The following references are of record in the file of this patent:

#### UNITED STATES PATENTS

| Number    | Name          | Date          |
|-----------|---------------|---------------|
| 2,502,030 | Scheiderbauer | Mar. 28, 1950 |